

Patented July 13, 1926.

1,592,302

# UNITED STATES PATENT OFFICE.

ZAY JEFFRIES AND ROBERT S. ARCHER, OF CLEVELAND, OHIO, ASSIGNORS TO AMERICAN MAGNESIUM CORPORATION, OF NIAGARA FALLS, NEW YORK, A CORPORATION OF NEW YORK.

## HEAT TREATING MAGNESIUM ALLOY.

No Drawing.

Application filed July 18, 1922. Serial No. 575,782.

Our invention relates to the heat treatment of magnesium base alloys, that is, those in which the principal metal is magnesium, and has among its objects the improvement of certain of the physical properties of such alloys and particularly the hardness and strength.

In a copending application, S. N. 507,766, filed October 14, 1921, we have described the heat treatment of magnesium base alloys, to improve certain of their physical properties, such as the plasticity or strength.

Our present discovery is preferably used in connection with that process, although it is not so limited, but is otherwise susceptible of general application. Generally speaking, the process comprises subjecting magnesium base alloys to heat treatment at a temperature preferably of approximately 150 degrees C. for an extended period of time. Considerable variation is permissible in the temperature for securing the desired changes in the characteristics of the treated metal and accordingly it can be as low as 125 degrees C. and as high as 300 degrees C. If the temperature of treatment is too low, changes in the characteristics of the metal will not occur or will require a period of time too long for commercial practice. On the other hand, if the temperature of treatment is too high, there is danger of not obtaining the desired hardness; either that or temporarily obtaining it, but passing later into a softer condition.

The process is not limited to any definite magnesium base alloy, although certain alloys are found to be particularly susceptible to improvement by treatment of the character described. An investigation of the alloys of magnesium with aluminum has shown that when the content of aluminum is 6% or less, the hardening which is obtained is insignificant. With an aluminum content of 8% or more, improvement results from the treatment described, the effect increasing with the content of aluminum at least up to about 12% aluminum. With alloys containing 12% aluminum, the amount and rate of hardening are found to be the greatest.

Alloys containing 4% aluminum and 4% zinc have also been found to be hardened by this heat treatment.

On the other hand, the presence of calcium in such alloys beyond a certain amount in-

hibits hardening. It is sometimes desirable to use calcium in connection with casting of the metal to prevent burning of the magnesium during both melting and casting of the metal and also during higher temperature heat treatments. In treating castings according to our process, we find that the chief effect of calcium up to 0.5% is to decrease the rate of hardening rather than the ultimate hardness.

In the practice of our process, it is desirable that the alloy be in proper receptive condition before the application of the low temperature heat treatment, and while prior heat treatment at a temperature of 400-440 degrees C. as described in our copending application, is preferable it is not entirely necessary that these precise heat treatments be applied as it is possible that the process of manufacture may be such that the alloy is left in a condition susceptible to our process without the necessity of the previous heat treatment.

As we have described our process, the treatment is applied as a distinct operation and is essentially a heating operation applied after the alloy has cooled from the temperature of fabrication or other processes involving the application of heat.

The same improvement in the properties of the metal may be obtained, however, by so regulating the rate of cooling from a high temperature that the metal will remain in the low temperature range for a suitable period of time.

The rate or character of cooling of the alloy from the temperature at which the hardening treatment is carried out is of practically no importance from the standpoint of hardness or increased strength.

Some of the different applications of our process may be illustrated by the following examples:

*Example 1.*—A piston was cast in an iron mold from an alloy containing 12% aluminum, the balance being nearly pure magnesium. After the casting had cooled to the ordinary temperature, it was found to have a Brinell hardness of 71. It was then subjected to a heat treatment process as described in our copending application, which consisted in heating for a period of 15 hours at 420 degrees C. and quenching in water. The Brinell hardness was then

found to be 66. The piston was then given a heat treatment of the character herein set forth and consisting in heating for a period of 40 hours at a temperature of 150 degrees C. At the end of this treatment, the piston was allowed to cool in air to room temperature. The Brinell hardness was then found to be 111.

*Example 2.*—An alloy of magnesium with 10% aluminum was extruded into rod  $\frac{1}{2}$  inch in diameter. This rod was found to possess the following physical characteristics: tensile strength 47,600 pounds per square inch, elongation 7.3% and Brinell hardness 70. Some of this rod was heated for  $\frac{1}{2}$  hour at 420 degrees C. and quenched in water. The physical characteristics were then: tensile strength 49,600 pounds per square inch, elongation 10.6% and Brinell hardness 58. Some of this heat treated rod was then subjected to a hardening treatment at 150 degrees for 15 hours. The hardness and strength were then found to have been markedly increased, as shown by the following values: tensile strength, 60,450 pounds per square inch, elongation 2.7% and Brinell hardness 91.

*Example 3.*—An alloy containing 4% aluminum and 4% zinc was extruded into rod  $\frac{1}{2}$  inch in diameter. Its Brinell hardness was found to be 60. After heating for  $\frac{1}{2}$  hour at 420 degrees C. and quenching in water, the Brinell hardness was 54. Some of this heat treated rod was then reheated for 15 hours at 150 degrees C. after which its Brinell hardness was found to be 73.

*Example 4.*—A 10% aluminum alloy in the extruded condition had a tensile strength of 47,600 pounds per square inch, with an elongation of 8.3% and a Brinell hardness of 71. Some of the rod was subjected to a hardening treatment, consisting in heating for 15 hours at 150 degrees C. after which it was found that the Brinell hardness was increased to values ranging from 80 to 94. One particular test bar had a tensile strength of 56,600 pounds per square inch, with an elongation of 2.7% and a Brinell hardness of 74.

*Example 5.*—The Brinell hardness of the piston as cast was 71. After the application of our process as described in Example 1, the hardness was increased to 111. The piston was then reheated for a period of 2 hours at 420 degrees C. If quenched from this temperature, the hardness would have been approximately 66. Instead of quenching, the piston was allowed to cool in air. During this cooling it was, of course, subjected to a certain sojourn in a temperature range suitable for hardening. After cooling to room temperature, the Brinell hardness was found to be 80.

*Example 6.*—A piece of 12% aluminum

alloy was heated in the as cast condition to 150 degrees C. and was found to harden. The rate of increase in hardness was much slower than in the case of specimens quenched in water from 420 degrees C. and the maximum hardness reached was lower than in the case of quenched specimens.

#### *Theory of operation.*

Aluminum is soluble in solid magnesium up to about 11 to 12% at the eutectic temperature of 435 degrees C. The solubility decreases as the temperature falls, the excess aluminum being precipitated in the form of a hard constituent. A magnesium alloy containing the aforesaid percentage of aluminum does not contain all of this aluminum in solution after normal solidification from the molten state. Alloys containing about 6% or more of aluminum when examined in the as cast condition are found to contain particles of the hard constituent, the amount increasing with the aluminum content. The process of solidification is such that the first material to freeze contains very little aluminum and as the freezing progresses the aluminum content of the metal freezing out increases. The resulting structure is an aggregate of grains of magnesium containing some aluminum in solution and partially surrounded by a network of the hard and brittle constituent which envelops the grains of the first mentioned material, the extent of the envelopment being somewhat in proportion to the aluminum content. Since the network is hard and strong, it imparts stiffness and hardness to the alloys and when not in too great quantity is a source of strength. Large amounts of the brittle network, however, causes brittleness of the alloys as a whole, with consequent diminished strength. It is, therefore, found that the maximum tensile strength of cast alloys occurs at about 7% aluminum although the hardness continues to increase up to at least 16% and probably beyond.

Although the network is completely soluble at the eutectic temperature, it is not possible to obtain complete solution merely by heating the alloy at this temperature. A diffusion process is necessary which requires considerable time. It is impracticable to heat treat at this temperature on account of the danger of melting the eutectic portions of the alloy before solution and diffusion are complete. As set forth in our copending application, we have found that a suitable temperature for alloys containing up to 12% aluminum is from 400 degrees to 440 degrees C. Prolonged heating at this temperature results in the solution of some of the brittle network and diffusion through the mass of the alloy, so that eventually a homogeneous solid solution is obtained. The solution and

diffusion of the hard network is found to improve the tensile strength and plasticity of the alloys. The Brinell hardness is in most cases slightly reduced. The elastic 5 limit and yield point may also be reduced. This heat treatment will hereinafter be referred to as the "solution heat treatment".

The solid solution obtained by the specified heat treatment which is unstable at lower temperature can be preserved by rapid cooling from the heat treating temperature. After quenching, changes in the characteristics of the metal, however, do not occur spontaneously, as in the case of some of 15 the light aluminum alloys, but require the application of heat, the necessary temperature for the specified alloys being from 125-300 degrees C.

In heat treating a solid solution at temperatures of 125 to 300 degrees C. the increase in hardness is understood to be attributable to the precipitation of the hard constituent in the form of very fine particles. The available evidence indicates that 20 this solid solution is made up structurally of crystalline magnesium in which some of the atoms are replaced by atoms of aluminum, the aluminum being in a state of atomic dispersion. When precipitation occurs, some 25 of the aluminum atoms and magnesium atoms become associated in a new space lattice, forming a new crystalline constituent of different physical properties, namely of 30 much greater hardness and less plasticity than the magnesium rich solid solution. The minute crystals of the new phase grow in accordance with the usual laws of crystal 35 growth on prolonged heating at sufficiently high temperatures. This heat treatment 40 will be referred to as the "precipitation heat treatment".

All evidence indicates that the greatest hardness is produced by the finest crystalline particles and that the hardness decreases as 45 these particles grow. It is therefore desirable to produce precipitation as completely as possible, but to avoid further growth of the particles as much as possible. This result is best accomplished by a long exposure 50 at a low temperature such as 150 degrees C. rather than by a brief exposure at a high temperature such as 300 degrees C.

While the maximum results from the precipitation heat treatment are obtainable 55 after the solution heat treatment, yet appreciable and important results from the precipitation heat treatment can be had, as a result of the nature of the cooling process in casting or otherwise fabricating the alloy, if a sufficient amount of aluminum has 60 been retained in the solid solution during cooling.

The change which takes place during the 65 precipitation treatment is an increase in hardness, elastic limit and tensile strength

with a decrease in plasticity. When the process is carried to completion the ductility is decreased to a marked extent, although this may not be true at all stages of the process. The process is therefore applicable in any case where it is desired to increase elastic limit, strength or hardness, providing the simultaneous loss of plasticity is not prohibitive, as for instance in the case 70 of pistons.

75 Experiments indicate that the necessary condition for hardening by the precipitation treatment is the presence of a supersaturated solid solution.

We claim:

1. The process of changing certain of the ultimate physical properties of magnesium base alloys comprising subjecting the metal to heat treatment at a temperature of approximately 150 degrees C.

80 2. The process of changing certain of the ultimate physical properties of magnesium base alloys comprising subjecting the metal to heat treatment at a temperature of 125 to 300 degrees C. to cause precipitation of a 85 hard constituent in the form of very small particles.

85 3. The process of heat treating magnesium base alloys to increase the hardness by subjecting the metal to a temperature of approximately 150 degrees C. for 15 to 40 hours.

90 4. The process of changing certain of the ultimate physical properties of magnesium base alloys comprising subjecting the metal to heat treatment at a temperature of 125 to 300 degrees C. for approximately 15 to 40 hours.

95 5. The process of increasing the hardness and strength of magnesium base alloys containing from 3 to 15% aluminum comprising subjecting the metal to heat treatment at a temperature of approximately 150 degrees C.

100 6. The process of increasing the hardness and strength of magnesium base alloys containing from 3 to 15% aluminum comprising subjecting the metal to heat treatment at a temperature of approximately 125 to 300 degrees C.

105 7. The process of increasing the hardness and strength of magnesium base alloys containing from 3 to 15% aluminum comprising subjecting the metal to heat treatment at a temperature of approximately 150 degrees C. for 15 to 40 hours.

110 8. The process of increasing the hardness and strength of magnesium base alloys containing from 3 to 15% aluminum comprising subjecting the metal to heat treatment at a temperature of approximately 125 to 300 degrees C. up to 40 hours.

115 9. The process of changing certain of the physical properties of magnesium base alloys by subjecting the metal to heat treat-

ment at a temperature of approximately 150 degrees C. for a period of time sufficient to cause substantial improvement in its hardness.

10. The process of changing certain of the physical properties of magnesium base alloys by subjecting the metal to heat treatment at a temperature of approximately 125 to 300 degrees for a period of time sufficient to cause substantial improvement in its hardness.

11. The process of changing certain of the physical properties of magnesium base alloys comprising subjecting the metal to heat treatment at a temperature of 400-440 degrees C. and thereafter subjecting the same to a temperature of approximately 150 degrees C. to increase its hardness.

12. The process of changing certain of the physical characteristics of magnesium base alloys containing aluminum, comprising subjecting the metal to heat treatment at a temperature of approximately 125° to 300° C. for a period of time sufficient to cause precipitation of a hard constituent.

13. The process of changing certain of the physical characteristics of magnesium base alloys containing aluminum, comprising subjecting the metal to heat treatment at a temperature of approximately 400° to 440° C. to secure a solid solution of magnesium and aluminum which will be supersaturated at room temperature and thereafter to heat treatment at a temperature of approximately 125° to 300° C. for a period of time sufficient to cause precipitation of a hard constituent.

14. An alloy containing magnesium as the principal metal and characterized by the

presence of a hard magnesium containing 40 constituent in the form of very small particles.

15. An alloy containing magnesium as the principal metal and containing aluminum from three to fifteen percent and characterized by the presence of a hard magnesium-aluminum constituent in the form of very small particles.

16. The process of treating magnesium base alloys to improve certain of the physical properties comprising subjecting the metal to heat treatment above 400 degrees C. and thereafter subjecting it for a period of time at a lower temperature to increase its hardness.

17. The process of improving certain of the physical properties of magnesium base alloys and particularly the hardness, comprising the heat treatment of a supersaturated solid solution of the metals at a temperature of approximately 125° to 300° C. for a period of time sufficient to cause precipitation of a hard constituent therefrom in the form of very small particles.

18. The process of improving certain of the physical properties of magnesium base alloys and particularly the hardness, comprising the heat treatment of a supersaturated solid solution of magnesium and aluminum at a temperature of approximately 125° to 300° C. for a period of time sufficient to cause precipitation of a hard constituent therefrom in the form of very small particles.

In testimony whereof we affix our signatures.

ZAY JEFFRIES.  
ROBERT S. ARCHER.